

20.1

NC

2,031,659

## UNITED STATES PATENT OFFICE

2,031,659

## PROCESS FOR MAKING SMOKELESS POWDER

Milton F. Lindsley, Jr., Kings Mills, Ohio, assignor, by mesne assignments, to E. I. du Pont de Nemours and Company, a corporation of Delaware

No Drawing. Application November 24, 1933,  
Serial No. 699,639

5 Claims. (Cl. 52—22)

This invention relates to a process of producing smokeless powder of a type adapted for use in small arms ammunition and more specifically for shotgun shell. Smokeless powder may be 5 nitrocellulose, nitrocellulose colloided with nitroglycerine, or either of these two products treated with stabilizing compounds and materials adapted to influence the speed of burning and hence the ballistic properties of the powder. In most 10 cases the propellant powder used in the ammunition comprises a blend of two or more powders of the type specified.

The present invention relates primarily to a 15 process of producing grains of nitrocellulose suitable for use as a bulk powder and characterized by the property of being readily ignited. These nitrocellulose grains are however adapted for further treatment such as colloiding with nitroglycerine, so the secondary aspect of the invention 20 resides in the process of colloiding these grains with nitroglycerine. The nitrocellulose grains colloided with nitroglycerine may then be treated for stabilization or for the purpose of further modifying the speed of burning or ballistic 25 properties.

The primary and secondary aspects of the invention as described are inter-related in that the first step or process of forming the nitrocellulose grains provides a product peculiarly adaptable for 30 the second step of colloiding the grains with nitroglycerine.

The starting material is nitrocellulose which 35 has been reduced to a physical fineness of such degree that most of it passes a fifty mesh sieve and all of it passes a forty mesh sieve. This nitrocellulose is placed in water and the entire remainder of the process takes place in closed vessels under water. This handling of the nitrocellulose provides the greatest margin of safety.

40 The finely divided nitrocellulose under water is pumped into a container in which it may be heated and agitated to controllable degrees. The agitation provides a suspension of the nitrocellulose in the water. Into this container or cooker is 45 pumped a mixed solvent for the nitrocellulose comprising one solvent which is miscible with the water and one which is not. A mixture of acetone and amyl acetate constitutes an appropriate 50 mixed solvent.

The mixed solvent is then agitated in the cooker 55 with the suspended nitrocellulose. The acetone, being miscible with both the water and the amyl acetate, divides between them, some being in aqueous solution and some in solution in the amyl

acetate. The agitation produces a multitude of small globules of amyl acetate containing acetone in the solution of acetone in water. These small globules bring about an agglomeration of the suspended nitrocellulose particles which are dissolved by the globules. The solvents are then distilled off by the application of heat.

The function of the acetone is to control the density of the nitrocellulose grains formed by the agglomeration of the nitrocellulose particles. 10 Acetone, methyl acetone and similar solvents have the property of leaving nitrocellulose in porous condition when expelled from the nitrocellulose by heat. The process therefore produces grained nitrocellulose which may then be screened and 15 used as finished bulk powder after supplemental finishing processes. If it is desired, however, that the grained nitrocellulose be colloided with nitroglycerine, it is again suspended in water by agitation in the cooker and nitroglycerine pumped 20 very slowly into the cooker.

25 Preferably the nitroglycerine has incorporated in it a substance to reduce the hazard of explosion, such as benzol. When the benzol strikes the water in the cooker, most of it floats off on the surface so it is to be observed that the benzol is used for the purpose of reducing danger of explosion solely and plays not part in the colloiding action.

The suspended nitrocellulose grains are agitated until the desired quantity of nitroglycerine 30 has been pumped slowly into the cooker. Then the benzol is distilled off and the heating continued for a period of from eight to twenty-four hours at a controlled temperature such as 185° F. 35 The purpose of this continued heating is to cause the solvent to penetrate and completely colloid with the entire nitrocellulose grain so that a hard, homogeneous product is produced. The quantity of nitroglycerine is chosen in relation 40 to the quantity of nitrocellulose so that the entire grain may be colloided and still a hard, stable grain be produced. The porousness of the nitrocellulose grain facilitates the complete colloiding 45 thereof. If the colloiding were less than complete, the nitrocellulose grains would tend to be jell-like or sticky on their surfaces.

While still in aqueous suspension, the grain 50 may be treated further with an explosive deterrent such as dinitrotoluene, with other materials adapted to impart specific ballistic properties, and with stabilizers.

It will, of course, be understood that the components of the mixed solvent used in forming 55

the nitrocellulose grains may be other than acetone and amyl acetate. For instance, in place of the acetone, one may use methyl acetone, ethyl ketone, ethyl ketol, propyl ketol and similar low boiling point solvents of the ketone type. In place of the amyl acetate, one may use butyl acetate, ethyl acetate, and similar water immiscible nitrocellulose solvents. The water miscible solvent may comprise 10 to 50% and the water immiscible solvent 90 to 50% of the mixed solvent employed.

However, in accordance with this invention, one component of the mixed solvent must be highly volatile and miscible both with the other solvent and with water. The other solvent must be immiscible with water so that it forms minute globules in the water upon agitation.

Likewise, materials other than benzol, such as gasoline and similar low boiling distillates may be used for rendering the nitroglycerine less dangerous to handle. For the purpose of assisting the skilled in the art in practicing this process, the following detailed description of the process is provided:

800 pounds of finely divided nitrocellulose is agitated with

200 gallons of water, in a closed cooker.

30 gallons amyl acetate, 20 gallons of acetone and 100 gallons of water are agitated together 30 in an open tank.

The contents of the open tank are pumped into the cooker. Agitation in both containers is continued during this period and is also continued in the cooker during the remainder of the process.

As soon as the finely divided nitrocellulose is formed into proper sized particles, heat is applied causing the volatile solvents to be stillled off into a condenser, which discharges into the open agitated tank, completing the graining cycle. 430 pounds of nitroglycerine (20% nitro-glycol) containing 240 pounds of benzol is slowly added to the suspended powder grains which are again placed in the cooker. The temperature during 45 this period is held at approximately 75° C. Heat is applied driving off the benzol, which is condensed, and collected.

Agitation is continued and the temperature is held between 75° and 80° C. until the powder 50 grains are quite hard. This takes from eight to twenty-four hours.

The grained powder is chilled and then is discharged into suitable containers.

Having described my invention, I desire to be 55 limited only by the ensuing claims:

1. A process of forming grains of nitrocellulose suitable for bulk powder from finely divided nitrocellulose, said process, comprising, the step

of suspending the finely divided nitrocellulose in water and agitating said suspension in the presence of a mixed solvent comprising one component which is a solvent for a nitrocellulose and which is miscible with water, and another component which is a solvent for the nitrocellulose but is not miscible with water, and then driving off said solvents. 5

2. A process of forming grains of nitrocellulose suitable for bulk powder from finely divided nitrocellulose powder said process comprising the step of suspending the finely divided nitrocellulose powder in water and agitating said suspension in the presence of a mixed solvent comprising acetone and amyl acetate, and then driving 10 off said solvents. 15

3. A process of forming grains of nitrocellulose suitable for bulk powder from finely divided nitrocellulose, said process, comprising, the step of suspending the finely divided nitrocellulose in 20 water and agitating said suspension in the presence of a mixed solvent comprising 40% acetone and 60% amyl acetate by volume, and then driving off said solvents.

4. A process of forming grains of nitrocellulose 25 from finely divided nitrocellulose, said process, comprising, the step of suspending the finely divided nitrocellulose in water and agitating said suspension in the presence of a mixed solvent comprising one component which is a solvent for 30 a nitrocellulose and which is miscible with water, and another component which is a solvent for the nitrocellulose but is not miscible with water, then driving off said solvents, and then agitating the nitrocellulose grains so formed in aqueous 35 suspension in the presence of nitroglycerine in quantity sufficient to colloid each grain in entirety.

5. A process of forming grains of nitrocellulose 40 from finely divided nitrocellulose, said process, comprising, the step of suspending the finely divided nitrocellulose in water and agitating said suspension in the presence of a mixed solvent comprising one component which is a solvent for 45 a nitrocellulose and which is miscible with water, and another component which is a solvent for the nitrocellulose but is not miscible with water, then driving off said solvents, then agitating the nitrocellulose grains so formed in aqueous suspension in the presence of nitroglycerine in quantity sufficient to colloid each grain in entirety, and then subjecting the nitrocellulose grains so treated with nitroglycerine to a controlled temperature for a period of from eight to twenty- 50 four hours to effect the complete colloiding of 55 the nitrocellulose grains with the nitroglycerine.

MILTON F. LINDSLEY, JR.